

## UNITED STATES PATENT OFFICE

LEWIS E. SAUNDERS AND LOWELL H. MILLIGAN, OF WORCESTER, AND MILTON F. BEECHER, OF HOLDEN, MASSACHUSETTS, ASSIGNEES TO NORTON COMPANY, OF WORCESTER, MASSACHUSETTS, A CORPORATION OF MASSACHUSETTS

## ABRASIVE PRODUCT AND METHOD OF MAKING THE SAME

No Drawing.

Application filed August 8, 1927. Serial No. 211,621.

This invention relates to abrasive products and more particularly to a grinding wheel made of abrasive grains bonded by a ceramic material.

A grinding wheel of this type is ordinarily made of abrasive grains, such as crystalline alumina or silicon carbide, united by a bond of ceramic material fired at a high temperature to form a vitreous or vitrified mass. Such a bond is ordinarily composed of a mixture of one or more clays, such as ball clay and slip clay, with feldspar, kaolin, flint and the like, and when matured is similar to porcelain or glass. There are a large number of bond compositions utilized in this field, depending upon the required grade of wheel hardness and the nature and size of the abrasive grains used, as well as the other desired characteristics of the wheel. The bond selection has heretofore depended to a large extent upon unscientific hit or miss methods, and in spite of many years of practical experimentation in trying out such bond compositions, the grinding wheels often display unexpected and undesired characteristics, and two wheels made of the same composition and supposedly by the same method may not be at all alike in their grinding properties. The grade of hardness of a wheel, or its apparent grade under grinding conditions, is measured largely by the strength with which the bond holds the abrasive grains in position under the stresses of grinding or of testing the wheel. A softer grade of wheel, having a low strength of bonding, ordinarily wears away faster during grinding than does a hard wheel. Yet, in spite of painstaking efforts by the wheel makers to produce uniform products, it is sometimes found that a wheel of supposedly harder grade wears away faster than one predetermined to be a softer wheel. Then again, some grinding wheels drop in their modulus of elasticity as they age, probably because of the gradual yielding to certain internal strains. Stability of the properties of the wheel is an important and desired characteristic.

A study of such problems as these shows that various factors heretofore neglected

must be considered. With crystalline aluminum oxide abrasives, for instance, the contamination of a bond of supposedly uniform composition by impurities and alumina from the abrasive must be considered. This is due to the fact that the vitrification process ordinarily requires a temperature of 1200° C. or higher, and it is found that at such a range of temperature the slag and glassy impurities present in the abrasive may exude at 55 the surface of the grain and mingle with the bond composition. In addition to slag exudation, the composition of the bond may be somewhat altered to a deleterious extent by 60 actual chemical attack of the molten bond on the surface of the abrasive grain. There may be as high as 32 times as much abrasive as there is bond in a given wheel mixture, hence the presence of but a small amount of 65 slag in the abrasive may materially affect the bond composition, and the effect will vary 70 depending upon the amounts of the ingredients employed. The amount of slag and alumina contributed by the abrasive to the bond will also depend on the temperature 75 and conditions of firing, as well as the particular abrasive and bond used. It is observed that but little slag exudes from the crystalline alumina abrasive at or below 80 1100° C. and it is therefore important to fire the wheels at temperatures appreciably below 1200° C. in order to control or to eliminate this condition. It is necessary, however, that with any given bond, a sufficient 85 firing temperature be used to give the bond enough fluidity so that it will come thoroughly into contact with the grain surfaces. It is observed also that decomposition of silicon carbide presents similar difficulties in 90 that the ingredients thereof enter and affect the bond composition.

Another difficulty lies in the fact that many of the vitrifiable bonds ordinarily employed in the manufacture of grinding wheels go through a swelling stage during the process of vitrification, and it is necessary that the wheel be porous enough so that the bond may swell into the pore spaces between the abrasive grains. This makes difficult the manufacture of wheels containing relatively large 95 100

amounts of bond. In the case of aluminous abrasive, this condition is probably due to the fact that the bonds ordinarily contain an iron compound, which is usually present as ferric oxid. This, and other ingredients acting to a lesser degree, dissociate or go through other chemical changes at the maturing temperature to which such bonds are subjected, with a resultant evolution of gas and a consequent swelling of the bond. This may take place rapidly if the maturing temperature is higher than 1200° C., and such bonds must be fired under such conditions that they go entirely through the swelling stage and ultimately subside as a glass; but the swelling may cause disarrangement of the abrasive grains, and otherwise change the wheel characteristics to a detrimental extent. Although modern grinding operations require long-lived fast cutting wheels which may be rotated at very high speeds, yet the problems above noted have made it difficult to manufacture such wheels, and particularly those made of grit sizes which are too large to pass through a screen of 16 meshes to the linear inch.

In the course of our investigation of such wheels we have observed a strained condition at the point of union between the glass bond and the grains of abrasive, and in many cases the development of fine cracks in the glass bond is readily apparent. These cracks may form either during the manufacturing operation, or as the wheel ages during use or disuse. The coefficients of expansion of aluminous abrasives and of various bonds have been studied, and we have found that the bonds ordinarily used do not have the same coefficients of expansion as the abrasive grains, and that consequently the customary operations of making a vitrified wheel result in setting up states of strain between such bodies. A difference in "fit" between the bond and the abrasive may strain the bond to the point where cracks develop in it, and in this condition the bond is said to be "crazed". The strength of a crazed bond is much less than that of the same bond in the uncrazed condition. This causes an excessive wearing away of the wheel during grinding, and may even result in actual rupture of the wheel by centrifugal force. These results become particularly noticeable if the wheel is made up of very coarse grain sizes.

We have also discovered that, in other cases, minute cracks or internal strains may be connected with the presence of crystals in the bond itself. It is probable that these effects develop because of differential coefficients of expansion between the crystals and the glass surrounding them, or because of the changes in the composition of the glass due to the separation from it of crystals of a different composition from the original glass. We have applied the term "crackling" to this

cracked condition of the bond when the crystals are involved. It is obvious that crystals of different kinds may act entirely differently in this respect, dependent on their chemical composition, size, expansivity, and other factors.

As an example of a raw bond in common use for making grinding wheels in which the abrasive is crystalline alumina, the following percentage composition may be cited:

|                  |       |
|------------------|-------|
| Silicon dioxide  | 58.0  |
| Aluminum oxide   | 15.9  |
| Ferric oxide     | 4.8   |
| Magnesium oxide  | 2.4   |
| Calcium oxide    | 4.5   |
| Sodium oxide     | 1.4   |
| Potassium oxide  | 2.5   |
| Titanium oxide   | 1.1   |
| Moisture         | 1.1   |
| Loss on ignition | 8.3   |
| Total            | 100.0 |

This composition matures to a glass at a temperature in the vicinity of 1200° to 1300° C.

An appreciable amount of iron oxide is present and this causes the bond to swell when fired, forming oxygen gas as the result of thermal dissociation above about 1175° to 1225° C. Such a bond first shrinks and sin-  
ters to a dense body, then it begins to soften and when sufficiently fluid it swells as gas is evolved, and finally it subsides to a dense black glass. When made up into a grinding wheel with crystalline alumina abrasive of the regular variety, which may contain about 95% of alumina and various impurities, such as ferric oxide, silica and titania, a wheel is produced which has many undesired characteristics. Such a wheel is to a certain extent unstable, in that its physical properties may change as it ages. The wheel may be soft in grade of hardness and weak compared with the strength that it should have. There is often found in such a glass bond a considerable development of plagioclase feldspar crystals and mullite crystals. Also, the bond in such a wheel is frequently found in a strained condition which results in crazing or crackling. This bond glass has a coefficient of expansion of about  $45 \times 10^{-7}$ , whereas crystalline alumina grains have an average coefficient of expansion of about  $72 \times 10^{-7}$ . A bond glass of this type may contain some undis-  
solved material of the original raw mixture as well as crystals which have been formed from the materials of the bond, either alone or together with those substances contributed by the abrasive.

We believe that the feldspar crystals are particularly detrimental in their tendency to cause crackling, but that a small quantity of the fine mullite needles sometimes observed in such a bond are not deleterious. The strains in such a glass bond may be released and cause crazing and crack-

ling at any time from the period of firing the wheel to years later, and this formation of cracks may be accelerated by the presence of moisture, or perhaps may be started by shocks 5 or scratches or thermal changes as well as by other conditions which are incident to the storage and aging and use of the grinding wheel. These disadvantages are particularly noticeable in wheels having a grit size of 10 abrasive coarser than that which will pass through a screen of 60 meshes to the linear inch. The larger grain sizes cause the greater trouble, due primarily to the larger area of contact between the grain of abrasive and 15 the bond.

The chief objects of our invention are accordingly to overcome such difficulties and in particular to provide a method of making an abrasive product containing bonded granular abrasive material which will not swell detrimentally during the manufacturing operation or craze or crackle as it ages or is 20 used.

Further objects are to provide such bonding ingredients and to so carry on the manufacturing procedure as to obtain products of ceramic bonded granular material which avoid the undesirable characteristics specified, and in particular to provide grinding 25 30 wheels or other ceramic bodies of this type which are stable, and not swelled, crazed or crackled to a detrimental extent and which may be made in the extremely hard and soft grades throughout a wide range of grain sizes 35 and degrees of porosity.

With these and other objects in view, as will be apparent to one skilled in the art, this invention resides in the composition of matter as well as the process of making the article 40 45 herein described as covered by the claims appended hereto.

In accordance with our discoveries and as the result of our experimentation, we have found that a grinding wheel should be made up of such materials that the abrasive grains and the bond will have substantially the same coefficients of expansion throughout a long range of temperature change and especially below the temperatures of softening or annealing of the matured bond, it being noted that at high temperatures the bond is capable of permanently deforming and yielding to the strains set up as the body cools. If the abrasive grains and bond expand and contract alike, then the formation of internal strains at the surface of the grains will be thereby minimized. It is important that crackling as well as crazing be minimized and this is accomplished by utilizing such bond compositions and so carrying out the vitrification process as to minimize, in so far as possible, the formation within the bond of an appreciable amount of crystals of sizes and types which have been found to be deleterious. It is desirable that the bond be

cooled rapidly through the range in which crystals may form, and if desired the bond may be cooled slowly below this range during the annealing period. We also prefer to employ a bond for a grinding wheel, which is substantially insoluble under ordinary conditions of usage in the liquids employed to cool or lubricate the wheel and work. We have found that the bond should be so constituted that it will not swell detrimentally 70 during the firing operation and that the bond should mature at a temperature sufficiently low so that the abrasive ingredients will not contaminate the bond to any considerable extent. The temperature at which the bond should mature, if the abrasive is crystalline alumina, should be below 1200° C., and preferably below Seger cone 6, it being noted that the slag and other impurities in the alumina abrasive tend to come out but little at 75 80 temperatures below 1100° C.

A bond composition for each abrasive which has these desirable characteristics may be readily picked out by one skilled in the art in view of the above disclosure. As an 85 90 illustration of one bond which is serviceable for use with an abrasive consisting largely of crystalline alumina, we may employ a bond mixture of the following percentage composition:

|                |       |
|----------------|-------|
| Silicon dioxid | 55.0  |
| Aluminum oxid  | 11.4  |
| Ferric oxid    | 4.3   |
| Magnesium oxid | 2.8   |
| Calcium oxid   | 5.9   |
| Sodium oxid    | 6.0   |
| Potassium oxid | 2.6   |
| Titanium oxid  | 0.7   |
| Boron oxid     | 11.3  |
| Total          | 100.0 |

A glass made up of this composition is found to have a linear coefficient of expansion of about  $72 \times 10^{-7}$  and this coefficient of expansion remains, below about 550° C., substantially the same as the average coefficient of the crystalline alumina abrasive grains. Above temperatures in the vicinity of 650° C., the bond is sufficiently soft so that it may 110 permanently deform and relieve any strains that may tend to be set up. Slow cooling in the annealing range, between say 650° and 550° C., will remove strains from the glassy bond, although there is but little, if any, tendency for permanent deformation in this range. The bond does not crystallize, if cooled with sufficient rapidity through the crystal forming range or until the bond begins to set, and therefore it does not crackle, nor does it craze at the line of junction with the alumina grains, hence the formation of internal strains and cracks is either obviated or to a large extent minimized. The bond 115 120 matures to a relatively stable glass at tem- 125 130

peratures below 1175° C., and does not swell detrimentally during such firing. Grinding wheels made with it have a fine, clear, permanent ring. It may be explained that the 5 grade of a grinding wheel may be estimated to a certain extent by the ring or musical note of the wheel when struck by a hammer and that the clearness of the ring indicates the absence of cracks or detrimental flaws in 10 the wheel.

As an example of a grinding wheel made up with this bond, we may employ crystalline alumina grains in grit sizes from 24 to 36 which have a chemical analysis of 95.24 15 alumina, ferric oxide 0.74, silica 0.93, titania 3.09. One grade of hardness of wheel may be made by using one ounce of this bond per pound of abrasive and the mixture may be suitably wetted with water or a solution of 20 a temporary binding material, and the mass shaped to the desired wheel form by suitable operations after which it may be fired. A ceramist skilled in this art will understand how to carry on the process of manufacture 25 so as to obtain the desired results, the different stages being in general first firing to vitrify or mature the bond, then cooling rapidly through the crystal forming stage, then slowly to effect proper annealing, and then 30 cooling below the point of solidification of the bond to set the wheel ingredients permanently. A wheel of the above specified composition may be fired to Seger cone 4, or a temperature of approximately 1125° C. The 35 wheel is preferably cooled rapidly to about 800° C. and then slowly to about 600° C. where the bond is solid. Below that temperature the bond and alumina abrasive grains have the same rate of shrinkage as the wheel 40 cools.

The wheel formed of the bond formula above specified is very stable and highly insoluble. A microscopic examination shows the bond to be relatively free from deleterious 45 crystals and it matures at a temperature below the dissociation point of ferric oxide and below the temperature at which an appreciable amount of slag exudes from the abrasive grain into the bond. This bond shows 50 but little tendency to swell during the firing operation and it is capable of bonding very coarse abrasive grains, as large as No. 8 grit or coarser, and of producing a hard grade of wheel which has a high bond strength.

55 While the example above given shows the applicability of this new type of bond to hard-graded and coarse-grained wheels, it is evident that soft wheels and those made of the smaller grit sizes may also be made, it 60 being merely necessary to vary the relative proportions of the wheel ingredients as is well understood in the art. It will be understood that the process and the bond composition will be varied depending on the kind 65 of abrasive employed, the grit sizes, the size

and shape of the article, the type of furnace employed and various other factors, and that the process will be so carried out as to obtain the desired wheel structure. It will also be apparent that various other products 70 besides grinding wheels may be made in accordance with this invention, and the claims are to be given a broad interpretation to cover ceramic products having granular abrasive material bonded by vitrified or glassy materials, whatever purpose the abrasive grains 75 may be intended to serve. For example, an article made in accordance with this invention of ceramic bonded abrasive material, such as crystalline alumina, has various 80 characteristics inherent in the hardness, durability, and refractory qualities of the bonded mass and its separate ingredients, as well as other physical and chemical properties, whereby the bonded product may be employed as a safety tread, a porous plate, a refractory brick or other article adapted to withstand high temperatures, and for many other uses. In each of these articles, the 85 utility of the bonded mass is greatly increased by providing a bond which has substantially the same coefficient of expansion as that of the grain.

Having thus described the invention, what we claim and desire to secure by Letters Patent is:

1. The method of making an article of ceramic bonded granular material comprising the steps of mixing abrasive grains with a ceramic bond which when matured will have substantially the same coefficient of expansion below the annealing range of the firing operation as that of the abrasive grains and thereafter firing the mixture to vitrify the bond and unite the abrasive grains into 10 an integral body.

2. The method of making an article of ceramic bonded granular material comprising the steps of mixing abrasive grains with a vitrifiable bond which matures at a temperature below that at which the constituents of the abrasive will deleteriously affect the bond and which has substantially the same coefficient of expansion below the annealing range as that of the abrasive grains, and thereafter shaping an article therefrom and firing it to mature the bond and unite the abrasive grains into an integral body.

3. The method of making an abrasive article comprising the steps of mixing abrasive grains with a vitrifiable bond which is so constituted that it will mature below 1200° C. without appreciable swelling taking place, and which, when vitrified, has substantially the same coefficient of expansion below the annealing range as that of the abrasive grains, and thereafter firing an article shaped therefrom to mature the bond and unite the grains into a solid body.

4. The method of making an article of

- ceramic bonded granular material comprising the steps of mixing crystalline alumina grains with a ceramic bond especially adapted for such grains which in the solid vitreous state has substantially the same coefficient of expansion as that of crystalline alumina and thereafter firing the mixture under such conditions as will mature the bond into a glass which unites the grains into an integral body.
5. The method of making an abrasive article comprising the steps of mixing crystalline alumina abrasive grains with a ceramic bond which is capable of maturing to a glass substantially free from crystal development and having substantially the same coefficient of expansion in the solid vitreous state as that of the abrasive grains and thereafter firing the article under such conditions as will mature the bond to a glassy condition, substantially free from deleterious crystals.
6. The method of making an article of ceramic bonded granular material comprising the steps of mixing grains of crystalline alumina with a ceramic bond which has substantially the same coefficient of expansion as that of crystalline alumina and which when matured to a solid glass will not be crazed or in a badly strained condition caused by a differential expansion between the bond and the crystalline alumina grains and which will mature below a temperature of 1200° C. and thereafter firing the mixture under such conditions as will mature the bond into a glass which unites the grains into an integral body.
7. The method of making an abrasive article comprising the steps of mixing the abrasive grains with a ceramic bond which has substantially the same coefficient of expansion as that of the abrasive grains and is capable of maturing into an uncrazed glass at a temperature below 1200° C. without deleterious crystal development and thereafter firing the mixture to mature the bond and cooling it rapidly through the range of possible crystal development to minimize the formation of crystals.
8. The method of making an abrasive article comprising the steps of mixing crystalline alumina grains with a ceramic bond which is capable of maturing to a glass without swelling materially and which has substantially the same coefficient of expansion in the solid vitreous state as that of crystalline alumina and thereafter firing a mass shaped from such mixture under such conditions as will mature the bond and unite the grains into an integral structure.
9. An abrasive article comprising abrasive grains bonded by a glassy material which has softened sufficiently below 1200° C. to adequately bond the grains together, and which when solid, has substantially the same coefficient of expansion as that of the abrasive grains.
10. A grinding wheel comprising crystalline alumina grains bonded by a substance which has substantially the same coefficient of expansion as that of crystalline alumina below the annealing range of temperatures and which is stable during normal usage.
11. A grinding wheel comprising crystalline alumina grains united by a ceramic bond, in the form of a glass which has substantially the same coefficient of expansion as that of crystalline alumina below the annealing range of temperatures and does not contain a detrimental amount of crystals, said bond being neither crazed nor crackled.
12. A bonded article comprising refractory abrasive granular material united by a vitrified ceramic bond in the form of a glass which has substantially the same coefficient of expansion as that of the abrasive material when solidified and is so constituted and has been so fired that it is neither crazed nor crackled.
13. The method of making a ceramic article comprising the steps of mixing abrasive material with a vitrifiable bond which has substantially the same coefficient of expansion as that of the abrasive material and which is capable of being matured without developing a material amount of deleterious crystals, and thereafter firing the mixture at such a temperature and cooling at such a rate as to mature the bond to a substantially homogeneous glass which is not crackled or crazed and in which there is no detrimental crystal development.
14. A bonded article comprising granular abrasive material united by a bond which has been softened and solidified in position between the grains, said bond being so constituted that it has substantially the same coefficient of expansion as that of the abrasive material between the temperature of solidification of the bond and the normal temperature of use.
15. An abrasive article comprising abrasive grains united by an uncrazed and uncracked ceramic bond which have substantially the same coefficients of expansion throughout the normal range of temperatures below annealing, said bond being a low melting glass, substantially free from deleterious crystals, which is capable of being matured below the temperature at which the constituents of the abrasive will deleteriously affect the bond and at which swelling of the bond may take place.
16. An article of ceramic bonded granular material comprising abrasive grains of coarse size united by a glassy bond which have substantially the same coefficients of expansion, said bond being substantially uncrazed and not in a materially strained condition, as caused by differential expansion between the grains and the bond, and being

uncrackled and substantially free from deleterious crystals.

17. An article of ceramic bonded granular material comprising crystalline alumina grains united by a glassy bond which have substantially the same coefficients of expansion, said bond being substantially uncrazed and not in a materially strained condition, as caused by differential expansion between the grains and the bond, and therefore fitting the grains below the annealing range of temperature, and being uncrackled and substantially free from deleterious crystals, a portion of the grains being of a size which will not pass through a screen having more than 36 meshes to the linear inch.

Signed at Worcester, Massachusetts, this 6th day of August 1927.

LEWIS E. SAUNDERS.  
20 LOWELL H. MILLIGAN.  
MILTON F. BEECHER.

25

30

35

40

45

50

55

60

65